

July 4, 1950

W. E. BARDGETT

2,513,395

BORON-TREATED MOLYBDENUM STEEL

Filed Aug. 5, 1947



INVENTOR

WILLIAM EDWARD BARDGETT

BY *Frederick E. Harry*

ATTORNEY

## UNITED STATES PATENT OFFICE

2,513,395

## BORON-TREATED MOLYBDENUM STEEL

William Edward Bardgett, Sheffield, England, assignor to The United Steel Companies Limited, Sheffield, England, a British company

Application August 5, 1947, Serial No. 766,398  
In Great Britain July 18, 1946

Section 1, Public Law 690, August 8, 1946  
Patent expires July 18, 1966

8 Claims. (Cl. 75—123)

## 1

This invention relates to alloy steels and has reference to alloy steels containing boron.

It has been recognised that the addition to steels of one of the elements which can be taken into solid solution such as boron, silicon, molybdenum, chromium and nickel increases their depth hardenability and it has been suggested that the characteristic of depth hardenability can be improved by some combinations of these elements, for example a combination of boron and silicon.

The present invention, although involving alloy steels containing boron, is not concerned with hardenability as normally understood and in fact involves considerations in the reverse direction in that its object is to provide a steel which possesses high maximum and yield stress characteristics without introducing appreciable hardening characteristics.

My invention is based upon the discovery that although the addition of boron to mild steel has no appreciable effect on its mechanical properties, the addition of boron in the presence of molybdenum has a pronounced effect on the maximum stress and the yield stress without introducing marked hardening characteristics in the steel.

According to the present invention, therefore, I provide an alloy steel having these desirable characteristics of high maximum stress and yield stress by the addition to mild steel of boron and molybdenum, or in other words the addition of boron to low carbon molybdenum steels.

A steel according to the invention possesses a high yield point in the as-rolled or normalised condition and freedom from high hardness on rapid cooling such as normally occurs in welding.

Hitherto there has been difficulty in providing a high yield point weldable steel owing to the fact that in order to obtain high yield strength, the carbon content requires to be above that which is normally safe for easy weldability. The limitation placed on the carbon content on this account does not normally permit of a yield strength greater than about 23 tons per sq. in. During welding the parent material adjacent to the weld material undergoes a cycle of heating involving rapid cooling from a temperature above the critical temperature. The properties of this zone are very largely dependent on the hardening characteristics of the material, high hardness resulting in material which is relatively brittle and liable to crack either during the cooling operation or subsequently in service.

The improvement obtainable by the use of the

## 2

invention is illustrated by the results of a series of tests on  $\frac{1}{8}$  inch diameter bars which had been normalised at  $930^{\circ}$  C. of steels containing approximately 0.08% carbon, 0.42% manganese, and 0.25% silicon. The addition of 0.003% boron to a plain carbon mild steel of this composition had no substantial effect on the mechanical properties. However, when 0.003% boron was added to a steel of similar composition but containing also 0.60% molybdenum, the effect was striking, the maximum stress being raised from 28 tons/sq. in. to 41 tons/sq.in. and the yield stress from 16 tons/sq.in. to 34 tons/sq.in. The Izod impact value of all these steels was unchanged at about 100 ft. lbs. These results are directly opposed to the general conception that boron is only of appreciable benefit in steels of medium carbon content in the hardened and lightly tempered condition.

20 Of the low carbon, low alloy steels tested, only those containing molybdenum have been found to respond appreciably to the influence of boron in the normalised condition or normalised and tempered condition, the most beneficial results being obtained in plain molybdenum steel.

25 The effect of molybdenum in low carbon, boron treated steel in the normalised condition is not linearly related to the mechanical properties. Molybdenum contents of up to about 0.20% have

30 only a small effect on the properties, but between about 0.20 and 0.40% there is a marked increase in the yield stress and maximum stress. Beyond about 0.40% molybdenum any further effect is relatively smaller. This and other characteristics of the steels of the present invention are shown graphically in the accompanying drawing, in which the yield stress in tons per square inch of various steels is plotted against the percentage molybdenum content of the steel. The carbon and boron content of these steels and the heat treatment they had received were as follows:

| Curve | Carbon, Per Cent | Boron, Per Cent | Heat Treatment                                                |
|-------|------------------|-----------------|---------------------------------------------------------------|
| A     | 0.05             | 0.003           | Normalised $930/940^{\circ}$ C.                               |
| B     | 0.05             | 0.003           | Normalised $930/940^{\circ}$ C. and tempered $650^{\circ}$ C. |
| C     | 0.13             | 0.003           | Normalised $910/920^{\circ}$ C.                               |
| D     | 0.13             | 0.003           | Normalised $910/920^{\circ}$ C. and tempered $650^{\circ}$ C. |
| E     | 0.14             | 0.006           | Normalised $910/920^{\circ}$ C.                               |
| F     | 0.14             | 0.006           | Normalised $910/920^{\circ}$ C. and tempered $650^{\circ}$ C. |

55 A minimum yield strength of 30 tons per sq. in. can be obtained in a boron treated steel containing not less than about 0.40% of molybdenum

## 3

with only about 0.05% carbon. Higher yield stress and maximum stress are obtained by increase in carbon but it is found that in order to obtain satisfactory mechanical properties, the carbon content should not usually exceed about 1.5%. Similarly it is found that increases in the boron content from .003 to .006% has a beneficial effect on the yield stress and maximum stress, but further increase in the boron content to 0.010 per cent has a markedly deleterious effect on the yield stress and also on the notch impact value.

The major portion of our experiments has been carried out on steels in which the boron has been introduced by the addition of a silicon-calcium-titanium-aluminium-zirconium ferro-alloy containing boron, but similar results may be obtained by the use of aluminium and ferro-boron with silicon contents of less than 0.1%.

The range of composition which I have found to be effective for the purpose of our invention is as follows:

|            | Full range            | Preferred range          |
|------------|-----------------------|--------------------------|
| Carbon     | Percent<br>up to .20  | Percent<br>0.11 to 0.15  |
| Manganese  | Percent<br>up to 1.0  | Percent<br>0.40 to 0.60  |
| Silicon    | Percent<br>up to 1.0  | Percent<br>0.10 to 0.55  |
| Molybdenum | Percent<br>.20 to .70 | Percent<br>.40 to 0.60   |
| Boron      | Percent<br>up to .010 | Percent<br>.003 to 0.004 |

A steel of the preferred composition in  $\frac{5}{8}$ " diameter bar in the normalised condition gives a minimum yield stress of 30 tons per square inch, good ductility and toughness and freedom from excessive hardening on rapid cooling.

The freedom from excessive hardening of steel according to the invention is demonstrated by the following figures showing the hardness across welds made by single runs of mild steel electrode on normalised one inch diameter bars.

| Analyses |      |      |        | Hardness H <sub>D</sub> /10 |                              |
|----------|------|------|--------|-----------------------------|------------------------------|
| C        | Mn   | Mo   | B      | Parent Metal                | Heat affected zone (Maximum) |
| 0.07     | 0.37 | 0.61 | 0.003  | 180                         | 219                          |
| 0.11     | 0.44 | 0.62 | 0.003  | 208                         | 252                          |
| 0.18     | 0.53 | 0.62 | 0.0025 | 220                         | 265                          |

Another advantage possessed by the boron treated steel of the present invention is that in the normalised condition it is generally equal to normalised and tempered material and on this account special heat treatment following rolling is, in many cases at least, unnecessary.

Yet another advantage of the addition, in accordance with the invention, of boron to low carbon molybdenum steel is the marked increase in ductility at elevated temperatures revealed by stress to rupture tests. As an example, the effect of adding boron to a  $\frac{1}{2}$ % molybdenum steel, as shown by a 24 hour test at a temperature of 1000° F., was to increase the stress to fracture from 18 to 28 tons per square inch, the elongation from 16 to 20% and the reduction in area from 23 to 57%.

In order to provide corrosion resistance, such elements as chromium, phosphorus and copper may be added to the low carbon molybdenum-boron steel.

I claim:

1. A weldable high yield point boron treated molybdenum steel having a carbon content not

## 4

exceeding 0.20 per cent and containing manganese up to 1.00 per cent, silicon up to 1.00 per cent, molybdenum from 0.20 per cent to 0.70 per cent, boron present in effective amounts but not exceeding 0.010 per cent and the remainder iron.

2. A weldable high yield point boron treated molybdenum steel having a carbon content not exceeding 0.20 per cent and containing manganese up to 1.00 per cent, silicon up to 1.00 per cent, molybdenum from 0.20 per cent to 0.70 per cent, boron present in effective amounts but not exceeding 0.010 per cent, and the remainder iron normalised by heat treatment.

3. A weldable high yield point boron treated molybdenum steel having a carbon content not exceeding 0.20 per cent and containing manganese up to 1.00 per cent, silicon up to 1.00 per cent, molybdenum from 0.20 per cent to 0.70 per cent, boron present in effective amounts but not exceeding .010 per cent, usual corrosion resisting constituents in conventional percentages, and the remainder iron.

4. A weldable high yield point alloy steel having a carbon content from 0.11 to 0.15 per cent, manganese from 0.40 to 0.60 per cent, silicon from 0.10 to 0.55 per cent, molybdenum from 0.40 to 0.60 per cent, boron from 0.003 to 0.004 per cent, and the remainder iron.

5. A weldable high yield point alloy steel having a carbon content from 0.11 to 0.15 per cent, manganese from 0.40 to 0.60 per cent, silicon from 0.10 to 0.55 per cent, molybdenum from 0.40 to 0.60 per cent, boron from 0.003 to 0.004 per cent, and the remainder iron and usual corrosion resisting constituents in conventional percentages.

6. A weldable high yield point boron-treated molybdenum steel having a carbon content not exceeding 0.20 per cent and containing manganese up to 1.00 per cent, silicon up to 1.00 per cent, molybdenum from 0.20 per cent to 0.70 per cent, boron from 0.0025 to 0.010 per cent, and the remainder iron.

7. A weldable high yield point boron-treated molybdenum steel having a carbon content not exceeding 0.20 per cent and containing manganese up to 1.00 per cent, silicon up to 1.00 per cent, molybdenum from 0.20 per cent to 0.70 per cent, boron from 0.0025 to 0.010 per cent, and the remainder iron normalized by heat treatment.

8. A weldable high yield point boron-treated molybdenum steel having a carbon content not exceeding 0.20 per cent and containing manganese up to 1.00 per cent, silicon up to 1.00 per cent, molybdenum from 0.20 per cent to 0.70 per cent, boron from 0.0025 to 0.010 per cent, usual corrosion resisting constituents in conventional percentages, and the remainder iron.

WILLIAM EDWARD BARDGETT.

## REFERENCES CITED

The following references are of record in the file of this patent:

## UNITED STATES PATENTS

Number Name Date  
2,283,299 Tisdale May 19, 1942

## FOREIGN PATENTS

Number Country Date  
160,792 Great Britain Aug. 25, 1921  
506,229 Great Britain May 24, 1939  
517,545 Great Britain Feb. 1, 1940

## OTHER REFERENCES

Metals and Alloys, October 1935, page 283.